

# UNITED STATES PATENT OFFICE.

ALBERT L. CLAPP, OF MARBLEHEAD, MASSACHUSETTS, ASSIGNOR TO THE METALITE COMPANY, OF AMESBURY, MASSACHUSETTS, A CORPORATION OF DELAWARE.

## WHITE LEATHER-BOARD AND PROCESS OF MAKING SAME.

1,302,513.

Specification of Letters Patent.

Patented May 6, 1919.

No Drawing.

Application filed April 27, 1916. Serial No. 94,060.

To all whom it may concern:

Be it known that I, ALBERT L. CLAPP, a citizen of the United States, and resident of Marblehead, county of Essex, and State of Massachusetts, have invented an Improvement in White Leather-Board and Processes of Making Same, of which the following is a specification.

My present invention is an improved 10 white leatherboard, made in a novel manner. In the manufacture of leatherboard as heretofore carried on, the various ingredients have necessarily resulted in the production of a colored product, usually of a 15 dark or brown appearance. Such dark colored effect was unobjectionable for many uses and purposes, particularly when used in the manufacture of light colored boots and shoes, building up heels, or the like. 20 Such prior leatherboard, however, could not be made white, nor whitened in any of the prior processes of manufacture, and it is an object of the present invention to produce a substantially white product of leatherboard 25 and in an economical, expeditious and commercial manner. One of the important uses of a white leatherboard is in the manufacture of white heels, quite recently popular in shoe manufacture, and my invention contemplates the manufacture of a leather- 30 board suitable for making heel lifts to be finished white. A peculiar difficulty in the manufacture of such white heelings is that the processes of manufacture and finishing 35 the heel included trimming and burnishing by high speed machines and therefore a great liability of damaging the leatherboard, by burning, etc., is present. I have discovered that my white leatherboard product may be made with a suitable admixture 40 which will preserve its whiteness and yet prevent the fibers from burning during such trimming or burnishing in the heel manufacturing steps.

45 In carrying out the process of manufacturing my white leatherboard, I prefer to employ a considerable amount of white waste paper of any sort or kind, as the principal stock to be beaten into pulp for the 50 white board. To this stock I add a considerable quantity of asbestos, which is also white and maintains this quality during the pulp beating. The asbestos, furthermore, is of special value in preserving the leather-

board fiber from burning when such board 55 is used in heel building, as above explained. I also add a preparation of white leather scraps, or chrome leather shavings and beat this mass into a pulp in an ordinary beater engine in the usual manner, utilizing as 60 much water as is necessary. In some instances it may be desired to add a sizing compound, although this is not always necessary. However, when the sizing is desired 65 in the leatherboard, I have discovered that a sea-weed size will not discolor the product, whereas ordinary materials, such as bark, peat, or other organic sizing, would discolor the board and render the same objectionable for use as a white leatherboard. 70 As a suitable charge for a beater, I use approximately 1000 lbs. of white waste paper, substantially 200 lbs. of asbestos fiber and a similar amount,—200 lbs.—of white leather scraps or chrome shavings, uniting these 75 thoroughly in a beater engine in the usual manner. To the charge thus prepared into white pulp, a suitable amount of sea weed sizing may be added when desired, and the pulp thus prepared is then formed into 80 sheets, either by running the same through on a wet machine, cylinder board machine, or may be pressed in a manner well-known in leatherboard manufacture.

The resulting product is a white leather- 85 board, substantially of uniformly white texture throughout, and of an extremely tough fibrous nature, suitable for use in the manufacture of white heels for boots and shoes, and to withstand the trimming and 90 burnishing operations of high speed heelng machines without danger of injury or burning. Moreover, the white leatherboard manufactured according to my novel process will receive a high degree of polish and 95 finish. The importance of this feature, in the manufacture of white heels for boots and shoes, will be appreciated when it is realized that heretofore white heels were made by covering the entire heel with a thin 100 layer of white leather, by cementing the leather thereto. This process involved great expense, had to be applied by hand and resulted in an unsatisfactory product, as the cemented covering for the heel easily peeled 105 off, especially if exposed to dampness.

A further feature of my present invention is that, for some purposes, especially

for the manufacture of white leatherboard for use in making boot and shoe heels, which must be able to withstand the "burning" incident to trimming, burnishing, etc., as 5 above explained, I can substitute French chalk for the asbestos ingredient. In such case a considerably larger amount of French chalk can be employed than the corresponding asbestos and considerably more sizing is 10 required to hold the chalk. I find that in making white leatherboard for boots and shoes in this manner, that simply white paper, French chalk up to as high as 30% of the mass, and from 10 to 15% of sizing can 15 be advantageously employed. One advantage of this formula consists in the cheapness and the fact that a more nearly pure white product may be obtained, which is often desirable to match the shoe uppers of 20 white kid, cloth, etc.

My invention is further described and defined in the form of claims as follows:

1. As an article of manufacture, white leatherboard comprising a proportion of 25 asbestos fiber.

2. As an article of manufacture, white leatherboard comprising white waste paper, asbestos fiber, and white leather scraps or chrome shavings.

3. As an article of manufacture, white leatherboard comprising white waste paper, asbestos fiber, and white leather scraps or chrome shavings, and a sea-weed sizing.

4. As an article of manufacture, white leatherboard comprising approximately the 35 materials and proportions following, viz: 1000 lbs. of white waste papers, 200 lbs. of asbestos fiber, and 200 lbs. of white leather scraps or chrome shavings.

5. The process of manufacturing white leatherboard, which is characterized by reducing to a pulp a mixture of white waste paper, asbestos, and white leather scraps or chrome shavings, and forming said pulp 45 into sheets.

6. The process of manufacturing white leatherboard, which is characterized by reducing to a pulp a mixture of white waste paper, asbestos, and white leather scraps or chrome shavings; adding thereto and thoroughly intermixing therewith, at some time during the process, a non-coloring sizing; and forming the stock thus obtained into sheets.

7. The process of manufacturing white leatherboard, which is characterized by reducing to a pulp a mixture of substantially 50 1000 lbs. of white waste paper, 200 lbs. of asbestos fiber, and 200 lbs. of white leather

scraps or chrome shavings, and forming the 60 stock thus obtained into sheets.

8. As an article of manufacture, white leatherboard comprising white waste paper, asbestos fiber, and white leather scraps or chrome shavings, all reduced to a finely com- 65 minuted state and thoroughly intermixed.

9. As an article of manufacture, white leatherboard comprising white waste paper, asbestos fiber, white leather scraps or chrome shavings and a non-coloring sizing, all re- 70 duced to a finely comminuted state and thoroughly intermixed.

10. As an article of manufacture, white leatherboard, comprising white fibrous stock, asbestos, and white leather scraps or chrome 75 shavings, all reduced to a finely comminuted state and thoroughly intermixed.

11. As an article of manufacture, white leatherboard, comprising white cellulose fibers, asbestos, and white leather scraps or 80 chrome shavings, reduced to a finely comminuted state and thoroughly intermixed.

12. As an article of manufacture, white leatherboard, comprising white fibrous stock, asbestos, white leather scraps or chrome 85 shavings, and a non-coloring sizing, reduced to a finely comminuted state and thoroughly intermixed.

13. The process of manufacturing white leatherboard, which is characterized by re- 90 ducing to a pulp a mixture of white fibrous stock, asbestos, and white leather scraps or chrome shavings; and forming the stock thus obtained into sheets.

14. The process of manufacturing white leatherboard, which is characterized by re- 95 ducing to a pulp a mixture of white fibrous stock, asbestos, and white leather scraps or chrome shavings; thoroughly intermixing with said pulp a suitable non-coloring sizing; and forming the stock thus obtained into sheets. 100

15. The process of manufacturing white leatherboard, which is characterized by re- 105 ducing to a pulp a mixture of substantially 1000 lbs. of white waste paper, 200 lbs. of asbestos fiber, 200 lbs. of white leather scraps or chrome shavings, and a quantity of non-coloring sizing; and forming the stock thus obtained into sheets. 110

In testimony whereof, I have signed my name to this specification, in the presence of two subscribing witnesses.

ALBERT L. CLAPP.

Witnesses:

JAMES R. HODDER,  
HAROLD J. CLARK.